# EUROPEAN PATENT SPECIFICATION

(11) **EP 2 405 040 B1**
(45) Date of publication and mention of the grant of the patent: **21.11.2012**
(21) Application number: 10007077.0
(22) Date of filing: 09.07.2010
(51) Int. Cl.: D04B 1/18, D02G 3/40, D03D 15/08, D03D 15/00, D03D 1/00, D04B 21/16

(54) **A penetration-resistant fabric manufacturing method which prevents yarn breakage during the manufacturing process**
Verfahren zur Herstellung eines penetrationsbeständigen Stoffes, das Garnbruch während des Herstellungsverfahrens verhindert
Tissu résistant à la pénétration, procédé de fabrication qui empêche la cassure des fils pendant le procédé de fabrication

(43) Date of publication of application: 11.01.2012
(73) Proprietor: Yu, King Yeung, Bldg., 216-218 Texaco Road, Tsuen Wan, N.T. Hong Kong (CN)
(72) Inventor: Yu, King Yeung, Bldg., 216-218 Texaco Road, Tsuen Wan, N.T. Hong Kong (CN)
(74) Representative: Karakatsanis, Georgios

(56) References cited:
- EP-A1- 1 754 814
- WO-A2-03/008683
- WO-A2-2010/045637
- US-A- 5 572 860
- US-B1- 6 212 914

## Description

### Technical Field

The present invention relates to a penetration-resistant fabric manufacturing method and more particularly pertains to a penetration-resistant fabric manufacturing method which prevents yam breakage during the manufacturing process.

### Background Art

WO 2010/045637 discloses a fusible bicomponent spandex which is prepared by a solution-spinning process such as dry spinning or wet spinning of spandex fibers including polyurethaneurea and polyurethane compositions, and which may prevent laddering, slippage of yarn, and enhance adhesion.

US5572860 discloses a fusible adhesive yarn in which spun core yarn, which is composed of elastic yarn and non-elastic short fiber assembly extending in the direction of the elastic yarn, and heat fusible yarn are twisted with each other in the same or opposite direction as or to that of the spun core yarn.

WO 03/008683 discloses a fabric formed by arranging a fusible yarn and melting said yarn to form a barrier.

The prior art has provided a tubular fabric for receiving underwire of brassiere which comprises a support yarn, an elastomeric yarn and a fusible yarn. The fusible yarn can be melted at a predetermined temperature and adhered to other yarns of the fabric to form a penetration barrier, and on cooling the melted fusible yarn produces a coating which has a temperature in excess of the predetermined temperature. The resultant tubular fabric is capable of preventing underwire protrusion by the penetration barrier formed by the fusible yarn, and the penetration barrier is durable as it would not be melted under normal circumstances, even when the fabric is subject to a washing machine for cleaning and drying.

However, fusible yarns are relatively fragile and easy to break. The fusible yarns are easily broken during the weaving process and thereby jamming the loom. Extra effort is required to handle the jamming of the loom and productivity Is therefore affected.

### Disclosure of the Invention

In view of the aforesaid disadvantages now present in the prior art, the present invention provides a penetration-resistant fabric manufacturing method which prevents yarn breakage during the manufacturing process.

To attain this, the penetration-resistant fabric manufacturing method according to claim 1 is proposed.

In a preferred embodiment, the support yarn is made from a polyamide such as Nylon. In other embodiments, the support yarn could be polyester. The inteitmisted comprises 22.2% by weight of the fusible yarn and 77.8% by weight of the support yarn. The fusible yarn and the support yarn are intertmisted by a two-for-one twister to form the intermisted yarn. The yarns are formed into a fabric in form of a tubular tape by weaving. The fabric comprises 22.1% by weight of intertmisted yarn. Apart from the intertmisted yarn the fabric may further comprise nylon. The fabric may be treated by heating during a dyeing process. The dyeing process comprises the steps of (i) steaming the fabric In a steamer at 102-105°C for dye fixing and (ii) drying the fabric in a drying unit at 80-110°C.

The fabric or tubular tape may be used for receiving underwire of brassiere, or for other purposes for all tapes.

The manufacturing process of the present invention is effective to prevent breakage of yarns during the weaving process. Intertmisting a fusible yarn and a support yarn to form a intertmisted yarn provides a stronger yarn in comparison to a conventional fusible yarn. Therefore, when feeding the intertmisted yarn into the weaving loom, the intertmisted yarn is less susceptible to breakage. As a result, loom jamming could be prevented and productivity is increased. For example, when a fabric Is formed by weaving a Nylon, a Lycra and a conventional fusible yarn model no. 56D/12F, the frequency of yarn breakage during the weaving process Is about once per 1.5 hours. However, when the manufacturing process of the present invention is applied, i.e. intertmisting a fusible yarn and a support yarn to form a intertmisted yarn first and then weaving the intertmisted yarn and an elastomeric yarn to form a fabric, the frequency of yarn breakage during the weaving process is reduced to about once per 12 hours. Best Mode for Carrying out the Invention

In a preferred embodiment, the present penetration-resistant fabric manufacturing method which prevents yarn breakage during the manufacturing process comprises the steps according to claim 1.

Particularly, the support yarn is made from a Nylon under model number 78/24/2 provided by Guangdong Xinhui Meida Nylon Co., Ltd. In other embodiments, the support yarn could be polyester. The fusible yarn in this embodiment Is model no. 56/12/1 provided by Lokpoon & Co., Ltd. The intertmisted yarn comprises 22.2% by weight of the fusible yarn and 77.8% by weight of the support yarn. The fusible yam and the support yarn are intertmisted by a two-for-one twister under model no. ASKV741 provided by Changzhou Peixing Textile Machinery Manufacturing Co., Ltd. to form the intertmisted yarn. The settings and operation of a two-for-one twister is readily available in the prior art and are therefore not described in detail herein. The yarns are formed into a fabric in form of a tubular tape by weaving. The weaving process is done by a weaving loom under model no. MULLER NF 27/6. The settings and operation of a weaving loom is readily available in the prior art and are therefore not described in detail herein. The fabric comprises 22.1% by weight of the intertmisted yarn. Apart from the intertmisted yarn, the fabric In this case further comprises nylon. The fabric is treated by heating during a dyeing process. The dyeing process comprises the steps of (i) steaming the fabric in a steamer at 102-105 ac for dye fixing and (ii) drying the fabric in a drying unit at 80-110°C. The dyeing, heating and cooling processes are well-known to a person skilled in the art and are therefore not described In detail herein.

The above embodiment is a preferred embodiment of the present invention. The present invention is capable of other embodiments and is not limited by the above embodiment. Any other variation, decoration, substitution, combination or simplification, whether in substance or in principle, not deviated from the scope of the present invention, is replacement or substitution of equivalent effect and falls within the scope of protection of the present invention.

## Claims

1. A penetration-resistant fabric manufacturing method which prevents yarn breakage during the manufacturing process, comprising the steps of:
(i) intertwisting a fusible yarn and a support yarn by a two-for-one twister to form an intertwisted yarn;
(ii) the intertwisted yarn and an elastomeric yarn are formed into a fabric;
(iii) treating the fabric by heating so that the fusible yarn melts and spreads over the fabric;
(iv) cooling the fabric to form a penetration barrier.

2. The penetration-resistant fabric manufacturing method which prevents yarn breakage during manufacturing of a fabric as in Claim 1, wherein the support yarn is made from a polyamide.

3. The penetration-resistant fabric manufacturing method which prevents yarn breakage during manufacturing of a fabric as in Claim 1, wherein the support yarn is Nylon.

4. The penetration-resistant fabric manufacturing method which prevents yarn breakage during manufacturing of a fabric as in Claim 1, wherein the support yarn is polyester.

5. The penetration-resistant fabric manufacturing method which prevents yarn breakage during manufacturing of a fabric as in Claim 1, wherein the intertwisted yarn comprises 22.2% by weight of the fusible yarn and 77.8% by weight of the support yarn.

6. The penetration-resistant fabric manufacturing method which prevents yarn breakage during manufacturing of a fabric as in Claim 1, wherein the fabric is formed into a fabric in form of a tubular tape by weaving.

7. The penetration-resistant fabric manufacturing method which prevents yarn breakage during manufacturing of a fabric as in Claim 1, wherein the fabric comprises 22.1 % by weight of the intertwisted yarn.

8. The penetration-resistant fabric manufacturing method which prevents yarn breakage during manufacturing of a fabric as in Claim 1, wherein the fabric comprises nylon.

9. The penetration-resistant fabric manufacturing method which prevents yarn breakage during manufacturing of a fabric as in Claim 1, wherein the fabric is treated by heating during a dyeing process.

10. The penetration-resistant fabric manufacturing method which prevents yarn breakage during manufacturing of a fabric as in Claim 9, wherein the dyeing process comprises the steps of (I) steaming the fabric in a steamer at 102-105 °C for dye fixing and (ii) drying the fabric in a drying unit at 80-110°C.

## Patentansprüche

1. Verfahren zur Herstellung eines durchdringungsfesten textilen Flächengebildes, das einen Fadenbruch während des Herstellungsprozesses verhindert, folgende Schritte umfassend:
(i) Verdrillen eines schmelzbaren Fadens und eines Stützfadens mit einer Doppeldraht-Zwirnmaschine, um einen verdrillten Faden zu bilden,
(ii) der verdrillte Faden und ein Elastomerfaden werden zu einem textilen Flächengebilde verarbeitet,
(iii) Behandeln des textilen Flächengebildes durch Erhitzen, sodass der schmelzbare Faden schmilzt und sich über das textile Flächengebilde ausbreitet,
(iv) Abkühlen des textilen Flächengebildes, um eine Durchdringungssperre zu bilden.

2. Verfahren zur Herstellung eines durchdringungsfesten textilen Flächengebildes, das einen Fadenbruch während der Herstellung eines Flächengebildes verhindert, nach Anspruch 1, wobei der Stützfaden aus einem Polyamid besteht.

3. Verfahren zur Herstellung eines durchdringungsfesten textilen Flächengebildes, das einen Fadenbruch während der Herstellung eines Flächengebildes verhindert, nach Anspruch 1, wobei der Stützfaden aus Nylon besteht.

4. Verfahren zur Herstellung eines durchdringungsfesten textilen Flächengebildes, das einen Fadenbruch während der Herstellung eines Flächengebildes verhindert, nach Anspruch 1, wobei der Stützfaden aus Polyester besteht.

5. Verfahren zur Herstellung eines durchdringungsfesten textilen Flächengebildes, das einen Fadenbruch während der Herstellung eines Flächengebildes verhindert, nach Anspruch 1, wobei der verdrillte Faden zu 22,2 Gew.-% den schmelzbaren Faden und zu 77,8 Ges.-% den Stützfaden umfasst.

6. Verfahren zur Herstellung eines durchdringungsfesten textilen Flächengebildes, das einen Fadenbruch während der Herstellung eines Flächengebildes verhindert, nach Anspruch 1, wobei das textile Flächengebilde durch Weben zu einem textilen Flächengebilde in Form eines röhrenförmigen Bandes geformt wird.

7. Verfahren zur Herstellung eines durchdringungsfesten textilen Flächengebildes, das einen Fadenbruch während der Herstellung eines Flächengebildes verhindert, nach Anspruch 1, wobei das textile Flächengebilde zu 22,1 Gew.-% den verdrillten Faden umfasst.

8. Verfahren zur Herstellung eines durchdringungsfesten textilen Flächengebildes, das einen Fadenbruch während der Herstellung eines Flächengebildes verklindert, nach Anspruch 1, wobei das textile Flächengebilde Nylon umfasst.

9. Verfahren zur Herstellung eines durchdringungsfesten textilen Flächengebildes, das einen Fadenbruch während der Herstellung eines Flächengebildes verhindert, nach Anspruch 1, wobei das textile Flächengebilde während eines Färbeprozesses durch Erhitzen behandelt wird.

10. Verfahren zur Herstellung eines durchdringungsfesten textilen Flächengebildes, das einen Fadenbruch während der Herstellung eines Flächengebildes verhindert, nach Anspruch 9, wobei der Färbeprozess die Schritte (i) des Dämpfens des textilen Flächengebildes in einem Dampfgerät bei 102 - 105 °C zur Farbfixierung und (ii) des Trocknens des textilen Flächengebildes in einer Trocknungseinheit bei 80 - 100 °C umfasst.

## Revendications

1. Procédé de fabrication de tissu résistant à la pénétration, qui empêche la cassure du fil pendant la fabrication d'un tissu, comprenant les étapes consistant à :
(i) torsader un fil fusible et un fil support par torsion de deux pour un pour former un fil torsadé ;
(ii) le fil torsadé et un fil élastomérique étant ensuite façonnés en un tissu ;
(iii) traitement du tissu par chauffage de manière à ce que le fil fusible fonde et s'étale sur le tissu ;
(iv) refroidissement du tissu pour former une barrière anti-pénétration.

2. Procédé de fabrication de tissu résistant à la pénétration pendant la fabrication d'un tissu, qui empêche la cassure du fil pendant la fabrication d'un tissu, selon la revendication 1, dans lequel le fil support est en polyamide.

3. Procédé de fabrication de tissu résistant à la pénétration pendant la fabrication d'un tissu, qui empêche la cassure du fil pendant la fabrication d'un tissu, selon la revendication 1, dans lequel le fil support est du nylon.

4. Procédé de fabrication de tissu résistant à la pénétration pendant la fabrication d'un tissu, qui empêche la cassure du fil pendant la fabrication d'un tissu, selon la revendication 1, dans lequel le fil support est du polyester.

5. Procédé de fabrication de tissu résistant à la pénétration pendant la fabrication d'un tissu, qui empêche la cassure du fil pendant la fabrication d'un tissu, selon la revendication 1, dans lequel le fil torsadé contient 22,2 % en poids de fil fusible et 77,8 % en poids de fil support.

6. Procédé de fabrication de tissu résistant à la pénétration, qui empêche la cassure du fil pendant la fabrication d'un tissu, selon la revendication 1, dans lequel le tissu est façonné en tissu sous forme d'une bande tubulaire par tissage.

7. Procédé de fabrication de tissu résistant à la pénétration qui empêche la cassure du fil pendant la fabrication d'un tissu, qui empêche la cassure du fil pendant la fabrication d'un tissu, selon la revendication 1, dans lequel le tissu contient 22,1 % en poids de fil torsadé.

8. Procédé de fabrication de tissu résistant à la pénétration qui empêche la cassure du fil pendant la fabrication d'un tissu, qui empêche la cassure du fil pendant la fabrication d'un tissu, selon la revendication 1, dans lequel le tissu contient du nylon.

9. Procédé de fabrication de tissu résistant à la pénétration qui empêche la cassure du fil pendant la fabrication d'un tissu, qui empêche la cassure du fil pendant la fabrication d'un tissu, selon la revendication 1, dans lequel le tissu est traité par chauffage pendant un processus de teinture.

10. Procédé de fabrication de tissu résistant à la pénétration qui empêche la cassure du fil pendant la fabrication d'un tissu, qui empêche la cassure du fil pendant la fabrication d'un tissu, selon la revendication 9, dans lequel le processus de teinture comprend les étapes consistant à (i) étuver le tissu dans une étuve à une température de 102 à 105° C pour fixer la teinture et (ii) sécher le tissu dans une unité de séchage à une température de 80 à 110° C.
